

Jan. 19, 1932.

M. N. RICH ET AL.

1,842,203

# ELECTRON EMITTING DEVICE AND METHOD OF PREPARATION

Filed May 19, 1926



INVENTOR  
MALCOLM N. RICH  
ERNEST A. LEDERER  
BY   
ATTORNEY

## UNITED STATES PATENT OFFICE

MALCOLM N. RICH AND ERNEST ANTON LEDERER, OF EAST ORANGE, NEW JERSEY, AS  
SIGNORS TO WESTINGHOUSE LAMP COMPANY, A CORPORATION OF PENNSYLVANIA

## ELECTRON-EMITTING DEVICE AND METHOD OF PREPARATION

Application filed May 19, 1926. Serial No. 110,047.

This invention relates to refractory metal filaments and more particularly to drawn thoriated-tungsten filaments suitable for use as cathodes in electron discharge devices.

5 In the prior art the addition of thoria to the tungsten filaments as prepared by the usual hot working methods, has been found to yield upon proper treatment, a low temperature electron emission of great utility, 10 which is attributed to the formation of a surface atomic layer of thorium metal upon the filament.

Various methods have been devised, heretofore, for the purpose of effecting a conversion of the thorium oxide content of drawn thoriated-tungsten filaments, to metallic thorium, so that the filaments might be advantageously used as cathodes in thermionic valves. One of the common methods here- 20 tofore employed, depends upon the addition of a carbon reducing agent to the filament in one form or another, for the purpose of effecting a reduction of the thorium oxide or suboxide content of the filament to thorium 25 metal, during a subsequent "seasoning" schedule given the filament after it has been mounted in the electron discharge device and the device suitably exhausted. The so-called "seasoning" of the filament is for the 30 purpose of enabling this added carbon to effect a reduction of the thorium oxide content of the filament, and the temperatures are so regulated that the liberated thorium 35 metal is diffused to the surface of the filament.

Such a method is described in application Serial No. 636,510 of Ralph E. Myers, filed May 3, 1923, entitled Evacuated devices and method of exhaust, and assigned to the West- 40 inghouse Lamp Company. Briefly, the method consists in heating the filament in a volatile hydrocarbon atmosphere at such a temperature and time interval, that decom- 45 position of the hydrocarbon is effected, and a deposit of carbon is formed upon the filament.

This addition of carbon to the filament has been found to be extremely advantageous in 50 the manufacture of high power electron discharge devices in which the plate electrode

is operated at a high temperature and has also been found advantageous in developing life and electron emission in cathodes used in low power devices under the conditions which have heretofore prevailed in their 55 manufacture. However, with improvements in the manufacturing conditions and with electrode materials now available for the manufacture of low wattage tubes, we have found that the addition of carbon is not only 60 unnecessary but improved results are obtained if the small amount of carbon accumulated during the drawing and swaging operations is substantially removed.

Recent investigation in radio tube construction has shown that the materials used in the construction of the plates and grids exert a profound influence on the life and maintenance of the thorium emission of the filament. This is due to what is known as 70 "back oxidation" effects, which are produced through the liberation of the oxygen contained in the oxide films on the plate and grid metal parts, under electronic bombardment, 75 which oxygen migrates to the filament and destroys the thorium film thereon.

When this oxide film on the plate and grid metal parts was removed by any suitable means, such as described in application Serial No. 18,958 of H. C. Rentschler, filed 80 March 28, 1925, entitled Electron discharge devices and assigned to the Westinghouse Lamp Company, or copending application Serial No. 85,016 of E. A. Lederer, et al, filed 85 January 30, 1926, entitled Electrodes for electron discharge devices, and assigned to the Westinghouse Lamp Company, it was found that it was not necessary to add carbon to the filament to obtain a formation of 90 thorium metal on the filament but on the contrary an excess quantity of carbon ap- 95 peared to retard or inhibit the decomposi- tion of the thorium constituent of the drawn thoriated-tungsten filament during so-called seasoning.

A plausible explanation of the beneficial effect of added carbon on the cathode in electron discharge devices employing plates which are not entirely free of oxide, such as the nickel plates heretofore almost univer- 100

sally used, is that the added carbon combines with the oxygen liberated from the plate and grid metal parts, and thus prevents the oxidation of the thorium metal film on the filament. The amount of oxygen or oxide in or on the plate and grid and the extent of carbonization of the cathode differ in each particular instance, depending on the treating conditions and can not be uniformly controlled. As a consequence, difficulty has been experienced in obtaining tubes having uniform operating characteristics. If there is an excess of oxide on the plate, loss of emission will result due to oxidation of the thorium content of the filament, whereas, if the carbon is in excess, loss of emission, due possibly to thorium carbide formation, is obtained.

It is an object of this invention to eliminate these variables incident to the manufacture of electron tubes and produce thorium activated cathode tubes having a high emissivity, long life and uniform operating characteristics.

Another object is to provide an activated thoriated-tungsten filament which is substantially free from deleterious carbon.

Another object is to provide an improved method of activating cathodes of the thoriated type whereby increased electron emission and life are obtained.

Other objects and advantages will herein-after appear.

In the performance of this invention we preferably employ drawn thoriated-tungsten filaments, as prepared by the usual hot working methods, such as the Coolidge method, described in Patent 1,082,933, although squirted filaments or tungsten-thorium alloy filaments which have been subjected to carbonization might similarly be treated, according to the method hereinafter described.

Briefly, the Coolidge method consists in "doping" tungsten oxide with a solution of thorium nitrate such as to yield after drying and igniting at a temperature sufficient to decompose the thorium nitrate, the desired percent of thorium oxide as a finely disseminated powder.

The tungsten oxide is then reduced in hydrogen, the metal powder compacted into slugs and the slugs suitably sintered to a coherent metal body in hydrogen.

Following the treating of the slug it is given the usual swaging and drawing operations, during which appreciable carbon absorption in the metal body is necessarily encountered, particularly in the higher temperature swaging operations, due to the carbonaceous lubricant and the gas furnaces employed in these operations.

In accordance with our invention the carbon addition heretofore employed to activate the filament is not only entirely dispensed with but we take the thoriated-tungsten fila-

ment at the conclusion of the drawing operation and remove therefrom a large proportion of the carbides and surface carbon obtained during fabrication, by subjecting the filament to the action of especially purified dry hydrogen, at a temperature and time interval necessary to effect such a removal. Obviously, such an operation varies with the size of filament, extent of carbonization, etc.

We have discovered that at temperatures ranging from 1500° to 2000° C., the carbides are decomposed rapidly by hydrogen with the removal of the carbon from the filament. If the hydrogen treatment is continued for too long a period of time or if the temperature employed is too high, good results will not be obtained, due possibly to partial reduction of the thorium compounds and while this is the ultimate object in activating the filament, it should be prevented until the filament is enclosed in the evacuated envelope since otherwise a portion of the thorium may be oxidized by contact with the atmosphere or if not oxidized, it will be volatilized out of the wire during the high temperature flash to which the wire must be subjected after mounting to develop full electron emission from the filament through the decomposition of the thorium compound content.

Preferably, the filament is hydrogen treated in a continuous manner before mounting in the electron discharge device or lamp, but if desired, the hydrogen might be introduced into the envelope and the filament heated therein by a passage of current therethrough, the hydrogen being subsequently exhausted.

After such treatment the filament may be incorporated into the electron discharge device and the same exhausted to a high degree, the electrodes being treated to remove as completely as possible, all occluded gases. The filament may then be heated to approximately 2850° C. to decompose the thorium compound, this treatment being continued only for a sufficient period of time to effect such reduction, since the thorium metal volatilizes away rapidly at this temperature.

While we do not desire to be limited to any particular theory regarding the activating action obtained by our treatment we suggest the following, as a possible explanation.

During the normal hot working of the wire it is subjected to strong carbonizing influence, due to the gas fired furnaces in which the wire is heated and the carbonaceous lubricant employed so that after the final drawing operation the thorium constituent of the wire may be, to a certain extent, converted to a carbide of thorium which must be later reduced in order to obtain an active thorium metal film on the filament for electron emission. Free carbon and tungsten carbide are also formed during these hot working operations and appear to retard the reduction of the thorium carbide during

the socalled "seasoning" of the filament. Under this theory, in order to obtain a complete reduction of the thorium carbide, it is first necessary to eliminate free carbon and tungsten carbide, or a substantial portion thereof, if an excess quantity thereof has been formed. It is highly desirable, however, that the thorium carbide or other thorium compound of thorium be not reduced prior to the seasoning of the filament, since otherwise a large proportion thereof will be volatilized from the cathode at the temperature to which it is necessary to heat the filament to obtain reduction of the main body of thorium compounds.

This selective decomposition of carbon, that is, the decomposition of tungsten carbide and removal thereof, together with the free carbon in the filament, without substantial reduction of the thorium compound appears to be accomplished by the hydrogen treatment. There are strong indications that in hydrogen the tungsten carbide is reduced more readily than the thorium compound so that if the temperature and period of the hydrogen flashing is correctly chosen, a very substantial proportion of the tungsten carbide will be removed without appreciable reduction of the thorium compounds. It further appears that in vacuo the thorium compounds are decomposed more readily as a result of the hydrogen treatment previously given, so that a large available supply of active thorium metal is produced in the filament.

We have found if the heating in hydrogen is conducted at too high a temperature or for too long a period, that the emission and life of the cathode is detrimentally affected, due possibly to the reduction of a large proportion of the thorium compound in addition to the tungsten carbide, the thorium metal so produced being volatilized away during the subsequent seasoning of the cathode, thus reducing the available thorium content.

In order that the invention may be more fully understood, reference will be had to the accompanying drawing in which the single figure illustrates diagrammatically apparatus which may be employed for treating the filament.

The thoriated-tungsten wire 1 as it comes from the final drawing operation, is wound on a reel 2 which may be mounted upon a suitable standard 3. The wire is withdrawn from the reel 2 and rewound on a second reel 4 mounted on a standard 5 and provided with suitable winding mechanism, such as a pulley 6 and a belt 7. A slight amount of tension is applied to the wire as it is drawn from the reel 2 by any suitable braking mechanism, such as a friction disc 8.

The wire on its passage from the reel 4 may pass through a tube or trough 9 open to the atmosphere and supported on standards

10. A mercury cup 11 at the entrance of the tube 9 makes electrical connection with the wire from a suitable source of current 12 through a conductor 13. A second mercury contact 14 completes the circuit through the wire and permits it to be heated during its passage through the tube 9. This heating of the wire in air or in an oxidizing atmosphere exerts a beneficial effect on the filament, rendering it soft and more pliable, and removes a large proportion of surface carbon.

The wire as it leaves the tube 9, is drawn through the hydrogen treating chamber 15 in which it is subjected to the treatment which forms the subject matter of this application. A stream of pure dry hydrogen is supplied to the chamber through the inlet pipe 16 and outlet pipe 17. Electrical connections for heating the wire during its passage through the hydrogen chamber is provided by mercury contacts 18 secured to the opposite end walls of the chamber. The mercury contained in contacts 18 seal the openings 19 in the end walls of the chamber and prevent the entrance of air therein. A pressure of hydrogen of approximately 7 millimeters of water is maintained within the chamber to create an internal pressure which assists in excluding the entrance of air therein. Heating current for the wire is supplied from the electrical source 12 by conductors 20 and 21, the voltage being adjusted by a suitable rheostat 22. A second rheostat 23 may be used to control the heating of the wire during its passage through the annealing chamber 9.

The temperature to which the wire should be heated during the hydrogen treatment depends upon the amount of carbon which it has absorbed during the wire drawing process and varies with different samples of wire. We have found, however, that the proper temperature necessary to accomplish the reduction of the carbides and removal of free carbon, may be determined by a simple mechanical test. Wire, as it comes from the drawing dies, tends to curl and kink. An arbitrary rate of speed may be selected, depending upon the size of the wire to be treated or distance between the mercury contacts 18 etc., which from previous experience has been found to be approximately the proper speed and the temperature then gradually raised by adjusting the rheostat 22 until the wire or filament comes out of the hydrogen chamber bright and clean and free from kinks and curls normally experienced.

In the apparatus described, the distance between the mercury contacts 18 was approximately 2 inches and the speed with which the wire was passed through the chamber varied from 1 1/2 to 3 inches per second depending upon the size of the wire. For wire size of approximately .6 mil which corresponds to a wire having a weight of .71 to .74 milligrams per 200 millimeter length, a speed of

2.3 to 3 inches per second was employed and the voltage across the ends of the section of wire undergoing treatment was adjusted between 55 and 70 volts. A gas flow of 3 to 7 cubic feet per hour was employed. In case of 1 mil wire at the speed given above, voltages between 35 and 48 volts were applied across the ends of the section undergoing treatment. In wire of approximately 1.6 mil a speed of 1½ to 2 inches per second was employed with a potential between the ends of the section undergoing treatment of 18 to 28 volts.

The flashing in hydrogen must be carefully conducted since it has been found that hydrogen exerts a profound embrittling effect on tungsten. It has been the practice, heretofore, to treat tungsten filaments in hydrogen, but such treatment has been for the purpose of annealing or recrystallizing the wire. Hydrogen was employed because it was believed to be inert with respect to the filament and the flashing done without regard to the physical effect of the absorbed hydrogen on the finished filament or the development of electron emission in the filament.

In accordance with the present invention the treatment in hydrogen is conducted for a very short period of time, the best results having been obtained when the wire was subjected to the reducing action of the hydrogen from about .5 to 1.5 seconds. This period of time is sufficient to effect a substantial removal of carbon from the filament with very little or no decomposition of thorium compounds. Moreover, the quantity of hydrogen absorbed by the wire during this short interval of heating is not sufficient to embrittle the same, and the recrystallization which takes place during this brief heat treatment is insufficient to materially reduce the strength of the filament.

We have further found it essential to employ a very pure dry hydrogen, since the presence of any moisture in the gas deleteriously effects the emission of the filament. The hydrogen employed in our process is preferably run through a pre-heater and through sulphuric acid, potassium hydroxide and phosphorus pentoxide driers to obtain the proper purity and dryness.

Following the usual process of mounting, sealing-in, exhausting, and flashing the getter of the electron discharge device, the filament is seasoned at a temperature in excess of 2500° C. and at approximately 2850° C. to effect a substantial conversion of the thorium compound content of the wire to thorium metal, in whatever manner it is accomplished, i. e., decomposition, dissociation, diffusion or reduction, and the thorium surface film built up on the filament in the usual manner at a temperature around 2200° C. For op-

eration the filament is heated to approximately 1700° C.

With electron discharge devices of the UX-199 type which employ filaments of approximately .6 mil diameter, the temperature for effecting the decomposition of the thorium carbide is obtained by applying a voltage of 11.5 to 12 volts. The temperature for diffusion of the thorium to the surface is obtained with 4.5 volts. The operating voltage is 3.3 volts.

With electron discharge devices of the UX-201-A type which employ a filament of approximately 1.6 mil diameter, the following seasoning procedure is employed. Decomposition of the thorium compound is obtained with 17 to 19 volts and diffusion to the surface with 7.5 to 8.0 volts. The normal operating voltage is 5 volts.

Electron discharge tubes employing filaments treated in accordance with our invention, taking precautions to remove a substantial proportion of the carbon content obtained during the drawing operation and observing good exhaust and oxide free plates and grids, give uniformly high initial electron emission and maintain such emission over a longer period of time than heretofore attained with tubes of similar design.

While this filament has been referred to in connection with oxide free plates and grids, it is not limited to use with such electrodes, but due to the fact that there is available more metallic thorium than has heretofore been obtainable, increased emission and life are procured with ordinary plate and grid materials. The oxide free plates and grids, however, tend toward the production of uniformity in the product, decreased shrinkage due to emission failures and increased efficiency and prolonged life of the device.

Forming gas, a non-explosive mixture of 10% hydrogen and 90% nitrogen, suitably dried and purified, may be advantageously used in this process instead of pure hydrogen, with slight adjustment in time and temperatures, to accommodate the process to the lower hydrogen content.

In order to render the filament more uniform in cross sectional area and to eliminate hot spots and irregularities therefrom, and to more effectively remove the carbon, the wire just prior to drawing or at any convenient point during the drawing operation, may have the surface scale of carbon, carbides, oxides, etc., removed and the wire rendered pliable by the treatment set forth in copending applications of Malcolm N. Rich, Serial No. 4140, filed January 23, 1925, entitled Pliable tungsten and method of producing the same; and Serial No. 65,881, filed October 30, 1925, Patent No. 1,663,564 entitled Refractory metal filament, both assigned to the Westinghouse Lamp Company.

Briefly, such process consists in making

the wire the anode of an electrolytic bath which evolves oxygen at the anode and isolating the cathode therefrom so that the hydrogen there liberated does not come in contact with the anode. This treatment removes the carbon and surface carbides and by eliminating the hydrogen from the wire, renders it extremely pliable at room temperatures. Wire subjected to this anodic treatment to remove the major portion of the carbon therefrom during drawing and then subjected to the careful hydrogen treatment specified above, after completion of the drawing has been found to give still greater life and maintenance for use in incandescent lamps than the hydrogen treatment alone and also to improve the product for use as cathodes in electron discharge devices. However, such anodic treatment is not essential to the production of excellent results but is merely augmentive in character.

While this invention contemplates the removal of carbon to assist in the activation of the filament, nevertheless, the addition of carbon to the filament as heretofore practiced does not necessarily preclude the development of some electron emission from the filament in an electron discharge device, particularly in power tubes in which high plate voltages are employed or in low voltage tubes if the device has been insufficiently evacuated, or if the plate and grid metal parts are not oxide free. However, the results obtained are not uniform. The amount of thorium metal reserve in the filament may be negligible, or it may be sufficient to maintain fairly good life.

On the other hand elimination of carbon from the filament does not necessarily expose the filament to unusual destruction from oxidizing influences, because of the fact that due to the greater thorium metal reserve formed in the filament by the hydrogen treatment, the normal oxidizing conditions encountered in electron discharge devices, are not sufficient to appreciably effect the initial electron emission of the filament nor the total operating life of the device.

Obviously, many changes may be made in the method described and other applications of the invention devised without departing from the invention and we do not desire to be restricted to the particular embodiments described except as limited by the appended claims.

What is claimed is:

1. The method of producing activated thoriated-tungsten cathodes which have been subjected to carbonizing influence, comprising heating the cathodes below 2000° C. in hydrogen to substantially remove the carbon and tungsten carbide content thereof and subsequently heating the filament in vacuo at about 2850° C. to decompose the thorium compounds therein.

2. The method of activating a thoriated tungsten cathode which comprises heating the cathode to from 1500° to 2000° C. in dry hydrogen for about one second and subsequently heating the cathode to about 2850° C. in vacuo for about one minute. 70

3. The method of activating, for electron emission purposes, a thoriated tungsten filament which has been subjected to carbonization which consists in removing surface carbon and other impurities from the filament prior to final drawing by electrolytic action and after final drawing heating the filament in dry hydrogen to from 1500° C. to 2000° C. for a brief period to further eliminate carbon therefrom and thereafter heating the filament in vacuo to temperatures approximating 2850° C. followed by a second and longer heating in the same vacuo to temperatures approximating 2200° C. 80 85

4. The method of activating a thoriated tungsten cathode which comprises effecting a removal therefrom of substantially all carbon except that which is combined as a thorium carbide compound by heating the cathode for a limited time interval in pure dry hydrogen to temperatures approximating 1500° C. to 2000° C. and subsequently heating the cathode in vacuo to temperatures approximating 2850° C. to effect a conversion 95 of the thorium carbide to thorium metal.

5. The method of activating a thoriated tungsten cathode which comprises effecting a removal therefrom of substantially all carbon except that which is combined as a thorium carbide compound by heating the cathode for a limited time interval in pure dry hydrogen to temperatures approximating 1500° C. to 2000° C. and subsequently heating the cathode in vacuo to temperatures approximating 2850° C. to effect a conversion of the thorium carbide to thorium metal and thereafter heating the cathode in the same high vacuo to temperatures approximating 2200° C. to diffuse the thorium to the cathode 100 105 110 surface.

In testimony whereof, we have hereunto subscribed our names this 18th day of May, 1926.

MALCOLM N. RICH.  
ERNEST ANTON LEDERER.

115

120

125

131